# EUROPEAN PATENT SPECIFICATION

(11) **EP 1 287 216 B1**
(45) Date of publication and mention of the grant of the patent: **19.09.2007**
(21) Application number: 01929875.1
(22) Date of filing: 11.05.2001
(51) Int. Cl.: E04B 1/94, B63B 3/68

(54) **FIRE-RESISTANT AND SOUND-ISOLATING PANELING SYSTEM FOR SHIPS INTERNAL AREAS LINING**
FEUERHEMMENDES UND SCHALLISOLIERENDES PANEELSYSTEM FÜR DIE INNENRAUMVERKLEIDUNG VON SCHIFFEN
SYSTEME DE PANNEAUTAGE IGNIFUGE ET INSONORISANT POUR LE REVETEMENT INTERNE DES NAVIRES

(30) Priority: 01.06.2000 GR 2000100186
(43) Date of publication of application: 05.03.2003
(73) Proprietor: Caretta Interiors S.A., 194 00 Koropi (GR)
(72) Inventor: NIKOLAIDIS, Galinos, 190 03 Markopoulo, Messogion (GR); STAMOULIS, Georges, 145 61 Nea Kifisia (GR); YANNOULIS, Panagiotis, 151 24 Maroussi (GR); AMIRADAKIS, Nikolaos, 190 03 Markopoulo, Messogion (GR); HASSIOTIS, Constantine, 152 37 Filothei (GR)
(74) Representative: Papaconstantinou, Helen
(86) International application number: PCT/GR2001/000023
(87) International publication number: WO 2001/096683

(56) References cited:
- EP-A- 0 846 813
- WO-A-97/21884
- WO-A-99/24682
- DE-A- 3 624 736
- DE-A- 19 546 979
- FR-A- 2 671 817

## Description

### FIELD OF THE INVENTION

The present invention relates to multi-layered, fire-resistant, sound-isolating panels for lining interior areas of ships with improved properties and better aesthetic appearance. Further, the present invention discloses a method to manufacture those panels.

### INTRODUCTION

The weight reduction of the materials, which are used for the construction of the ships accommodation areas, is more and more important for the weight reduction (transportation capability increase) and the satisfaction of the relative strict regulations for the modem passenger ships.

The use of prefabricated sections of the accommodation areas, so that the ships construction total time is reduced, is constantly increasing at today's extremely competitive environment of this industrial sector internationally.

The satisfaction of the more and more strict specifications of sound-isolation for the passengers' and crew's comfort, as well as the satisfaction of the more and more strict rules of the fire-resistance for the safety of the Life at Sea (SOLAS), is necessary.

### 1. GENERALLY

The present patent concerns the construction of various types of panels for the ships internal areas coating with layers of fire-resistant and sound-isolating materials, that hold in with multiple layers of Magnesium content.

The following especial characteristics constitute the originality of the patent:
a) Chemical composition (components specific percentages/Absence of Sulfur Magnesia) and production mode of the binding material.
b) Internal structure, connection and reinforcement of the panels layers.
c) Assembling methodology of these panels for the prefabrication, transportation and installation of various sections of the accommodation areas, so that, after their installation and modulation on the ships, they:
   1) Meet the strict specifications of sound-isolation
   2) Meet the strict specifications of fire-resistance
   3) The strength of these materials as well as the strength of the formed areas, during the extreme strain of the ships in the sea under the most sever conditions, is ensured.
   4) The weight reduction, in comparison with the conventional panels, is ensured.

### 2. VARIOUS PUBLICATIONS

a) The U.S. Pat. No. 3,098,062 refers to a lining type with layers, that consists of an internal inflexible element from metallic fibers and at least one surface layer of plaster. The fiber element is covered by a paper layer, which offers a nice surface for final sheathing (e.g. with color). The plaster's strength in fire is limited and the surface layer is soft and fragile.
b) The Belgian Publication Number 886.016 refers to a production method of a heat-insulating cast covering, which consists of magnesium oxide and magnesium chloride. This mixture can be combined with a kind of reinforcing material. More details on the application of this material, how the strength of the various constructions, where it is applied, is ensured, as well as the sound-isolation and the fire-resistance accomplished, is not mentioned.
c) The Patent Application Number WO 97/21884, which constitutes the closest prior art, refers to a lining panel that consists of one or two isolating layers.

The fire-resistant binding material contains:
magnesium chloride
magnesium sulfate
magnesium oxide
sodium silicate

Other times the basic element of the fire-resistant material is described to be the magnesium chloride, at a percentage up to at least 47% and other times the basic element of the fire-resistant material of the lining panel is the magnesium oxide, at a percentage up to 48,3%,

The use of the magnesium sulfate has many problems when the panels happen to be in conditions of increased relative moisture, in combination with low environment temperatures, during the production, but also during the transportation and after the installation at the ship.

The internal reinforcements of the lining panels are constructed by the same binding material, resulting in noise transfer and in not meeting the strict sound-isolation specifications.

The Publication also refers, without details, only to one binding of floor and wall, resulting in not knowing the fire-resistance of a complete system, that is a complete construction, with linings, partition walls, ceilings and doors.

### 3, PATENTS OBJECT

We have now unexpectedly found that by modifying the composition of the binding material a better sound-isolating and fire-resistant panel is obtained, which is also of reduced weight. In addition, the novel panel includes new or specially constructed components, which provide better aesthetic appearance and high strength, without compromising the sound isolating properties of said panel.

Accordingly, the present invention relates to a fire resistant and sound isolating panel for a ship's accommodation area, said panel having the features as defined in claim 1.

### 4. PATENTS PURPOSE

The purpose of the patent is achieved, firstly wit the layering and the internal structure of the panels, combined with the connecting, the prefabrication, as well as the transportation and the installation of the final construction of the accommodation areas sections, such as side linings partition walls, ceilings, doors, complete cabins, sanitary areas.

### 5. LAYERING AND INTERNAL STRUCTURE OF PANELS

This is achieved through the installation of various layers of glass-cloth as a support, a layer or layers of mineral fiber as an insulating material and multiple layers of binding material, which contains magnesium oxide, magnesium chloride, sodium silicate in proper percentages, so that after the solidification, the desired strength to fire is succeeded.

In FIG. 1, the multiple layering of a simple panel are shown. Layer I consists of a low density glass cloth, for the achievement of a perfectly smooth panel surface after the solidification and take out from the mold.

Layers 2 and 3 consist of a higher density glass cloth. Layer 4 consists of mineral fiber. Mineral fiber's strips are fitted alongside the small dimension of the panel. At certain distances, for the improvement of strength in compression and the satisfaction of strict sound insulation specifications, higher density strips of mineral fibers (7), immersed in and enriched with a binding material, are fitted in parallel with the high dimension of the panel and vertically to the surface level.

Layers 5 and 6 consist of glass cloth similar of the layers 2 and 3.

The described layers, combined with the multiple layers of binding material consist a system with excellent fire-resistant and sound-isolating result and a low weight.

### 6. COMPOSITION OF THE BINDING MATERIAL

Magnesium blent of MgO-MgCl2 improved by the addition of sodium silicate is used as the binding structural material of the panels.

For the preparation of the binding material, the following raw materials are used:
1. Magnesia (MgO), of 91-95% purity.
2. Magnesium Chloride (MgCl2), of 47% purity.
3. Sodium Silicate (SiO2:Na2O)
4. Water

The composition of the binding material during its application is the following:

| | |
|---|---|
| 1. Magnesia (MgO) | 33,33% |
| 2. Magnesium Chloride (MgCl2) | 24,24% |
| 3. Water glass | 2,02% |
| 4. Water | 40,40% |

The Magnesium Oxide, as shown at the composition, is the basic component of the mixture, with excellent Fire Resistance results.

The Magnesium Chloride increases the hardness of the mixture after the solidification and improves its resistance in fire, while the water glass acts as the binding mean.

The used Magnesia is coming from baking of magnesite of Evoias or of Vavdou Halkidikis.

The described binding material is particularly appropriate for panels that are constructed with the technique of cold compression.
PICTURE 1
   Lining Panels of 25 mm
   Front side of 2,5 mm composite plate composed of 3 layers glass fibre reinforced board (layers 1-3).
   Middle part of 20 mm mineral wool type "Rockwool Fire Slab 160" (layer 4).
   Back side of 2,5 mm composite plate, composed of 2 layers glass fibre reinforced board (layer 5-6).
   The panel is internal stoned with "Rockwool Marine Slab 200", embossed in surfaces composition, in a distance of 300 mm from each other.
PICTURE 2
   Ceiling Panel of 25 mm
   Ceiling panel, is made of the same construction layers according to Picture 1. The panels are joined together with a galvanized steel profile (80*20 mm) filled with "Rockwool Marine Slab 160" and screwed on a support galvanized top profile (80*40 mm).
PICTURE 3
   Lining Panels of 25 mm
   The panels are joint together with a separate piece of panel (80*20 mm), consist of "Rockwool Marine Slab 160" covered on both sides with 2,5 mm glass fibre reinforced board.
PICTURE 4
   Section of Lining Panel 25 mm
   25 mm lining panels are installed on board wit a joint galvanized steel profile, 25*25*25*1 mm at the bottom side.
PICTURE 5 & 6
   Ready Made Corners
   Special fabricated panels in various sizes and shapes to be joined with standard lining panels.
PICTURE 7
   Connection of Wall & Ceiling Panels
   To connect the wall and ceiling panels, a galvanized steel profile is used, fitted on the wall panel. The ceiling panel, reinforced with an inner galvanized Steel profile, is screwed at its final position.
PICTURE 8
   Partition Panels of 50 mm
   B-30 class bulkhead of 50 mm thick is made of mineral wool type "Rockwool Fire Slab 110" reinforced along edges with "Rockwool Marine Slab 200".
   The mineral wool is covered on both sides with 2,5 mm composite plate consisted of glass fibre reinforced board (same construction layers as Picture 1).
   The panels are joined together with a galvanized steel bar 40*2 mm.
PICTURE 9
   Partition Panels of 50 mm
   The 50 mm partition panel is internal stiffened with "Rockwool Marine Slab 200" embossed in surfaces composition at a distance of 300 mm from each other.
PICTURE 10
   A-60 Class Single Leaf Hinged Door
   The door blade is fabricated with "Rockwool Maine Slab 160" faced on both sides and in middle with 2,5 mm composite plate composed of glass fibre reinforced board.
   The leaf is internal stiffened with "Rockwool Marine Slab 200" of width 20 mm, embossed in surfaces composite in a distance of 300 mm from each other.
   Inner reinforcement steel edge profile and outer steel edges trim.
   Frame of 3 mm "Z" profile in mild steel.
   Total door thickness: 46 mm.
PICTURE 11
   B-30 Class Single Leaf Hinged Door
   The blade is fabricated with "Rockwool Marine Slab 160", faced on both outer sides and in the middle with 2,5 mm composite plate composed of glass fibre reinforced bond.
   The leaf is internal stiffened with "Rockwool Marine Slab 200" of width 20 mm, embossed in surfaces composite in a distance of 300 mm from each other.
   Inner reinforcement steel edge profile and outer steel edges trim.
   Frame from 1,5 mm steel profile.
   Total door thickness: 33 mm.

## Claims

1. A fire resistant and sound isolating panel for a ship's accommodation area, said panel comprising:
(a) a first external layer (2, 3) and a second external layer (5, 6), said first (2, 3) and second (5, 6) external layers being disposed on opposing sides of the panel,
(b) an internal layer (4) of insulating material comprising mineral fibre,
**characterized in that**
each of the said external layers (2, 3; 5, 6) consist of two glass cloth layers which are connected with a binding material, wherein said binding material comprises magnesia, magnesium chloride, sodium silicate and water and is free of magnesium sulphate; **in that** said internal layer (4) is connected to said external layers (2, 3; 5, 6) with layers of the same binding material;
and **in that** said panel further comprises:
(c) reinforcing means (7), comprising a plurality of reinforcing elements (7), for reinforcing the panel, said reinforcing means being disposed within the internal layer (4) and connecting the first (2, 3) and the second (5, 6) external layers; the reinforcing elements (7) consisting of an insulating material of a higher density mineral fiber (7), immersed in and enriched with a binding material, and
(d) an additional layer (1) of glass cloth of lower density than the density of the glass cloth layers (2, 3; 5, 6), said additional layer being disposed on an outside surface of the panel so that said additional layer (1) remains visible upon installation of the panel in the ship's accommodation area, said additional layer (1) being connected to the first external layer (2, 3) with the binding material.

2. The panel according to claim 1, wherein the binding material consists of 33.33% magnesia, of 91-95% purity, 24.24% magnesium chloride, of 47% purity, 2.02% sodium silicate, and 40.40% water.

3. The panel according to claim 1, wherein the glass cloth layers (2, 3; 5, 6) are connected to each other and to the internal layer (4) with multiple layers of the binding material, and wherein said additional layer (1) is provided with a surface suitable for coloring or is covered with a fire-resistant decorative coating that remains visible in the accommodation areas of the ship upon installation of the panel.

4. The panel according to claim 1, wherein said reinforcing means (7) are reinforcing strips fitted in parallel to the high dimension of the panel and vertically to its surface, said means being connected to the insulating material of the internal layer (4) and to the external layers (2, 3; 5, 6) of the panel by multiple layers of the binding material.

5. The panel according to claim 1, wherein said reinforcing means (7) comprises any other appropriate reinforcing material.

6. The panel according to claim 1, further comprising connecting means for connecting the panels to each other, to a floor area, to angular elements, or to general panel supports for installation of the panel on the ship.

7. The panel according to claim 1, wherein said panel has a thickness of 25 mm.

8. The panel according to claim 1, wherein the panel is a double thickness panel having a thickness of 50 mm, wherein the double thickness panel has a thick internal layer of insulating material.

9. A fire-resistant door made of panels according to any one of the preceding claims, comprising
(a) a first external inflexible layer (2, 3) and a second external inflexible layer (5, 6), said first and second external inflexible layers (2, 3; 5, 6) being disposed on opposing sides of the door, and an internal inflexible layer, each of said first (2, 3), second (5, 6) and internal layers comprising layers of glass cloth connected with a binding material;
(b) first and second internal insulating layers (4) comprising mineral fibre, said first and second insulating layers (4) being connected to said inflexible layers (2, 3, 5, 6) with the binding material, wherein the first internal insulating layer (4) is disposed between the first external inflexible layer (2, 3) and the internal inflexible layer, and the second internal insulating layer (4) is disposed between the second external inflexible layer (5, 6) and the internal inflexible layer; and
(c) a plurality of reinforcing elements (7) inserted into the first and second internal layers (4) and connecting the inflexible layers, said reinforcing elements (7) comprising an insulating material of high density mineral fibre immersed in and enriched with a reinforcing binding material;
wherein said binding material comprises magnesia, magnesium chloride, sodium silicate and water and is free of magnesium sulphate.

10. A method of constructing the panel of claim 1, which method comprises a step of lamination using a cold compression process,
**characterized in that**
said first external layer (2, 3) comprises a most external glass cloth layer (1) of lower density than the density of the other external glass layers;
**and in that**
said binding material comprises magnesia, magnesium chloride, sodium silicate and water and is free of magnesium sulphate.

11. A method for constructing a prefabricated or semi-prefabricated ship accommodation cabin, comprising
(a) providing a plurality of panels, comprising the panel of claim 1; and
(b) assembling the cabin from the panels.

12. A method for constructing a prefabricated sanitary unit for a ship, comprising
(a) providing a plurality of panels including the panel of claim 1; and
(b) assembling the sanitary unit from the panels.

13. A method for constructing a fire-protection class B-15 connection for connecting vacuum toilet systems, comprising
(a) providing a plurality of panels including the panel of claim 1; and
(b) assembling the connection from the panels.

14. A method for constructing ceiling recesses in a ship, comprising
(a) providing a plurality of panels including the panel of claim 1; and
(b) assembling the ceiling recesses from the panels.

## Patentansprüche

1. Feuerbeständiges and geräuschisolierendes Paneel für Schiffunterkunftsbereichen, wobei das genannte Paneel aufweist:
(a) eine erste äussere Schicht (2, 3) und eine zweite äussere Schicht (5, 6), wobei die genannten ersten äusseren (2,3) und zweiten äusseren (5,6) Schichten an entgegengesetzten Seiten des Paneels angeordnet sind,
(b) eine innere Schicht (4) aus Isolierstoff, der Mineralfasern aufweist,
**dadurch gekennzeichnet**
**dass** jede der genannten äusseren Schichten (2, 3·5,6) aus zwei Glastuchschichten besteht, die durch ein Bindemittel verbindet sind, wobei das genannte Bindemittel Magnesia, Magnesiumchlorid, Natriumsilikat und Wasser aufweist und kein Magnesiumsulphat enthalt-
**dass** die genannte innere Schicht (4) mit den genannten äusseren Schichten (2, 3· 5,6) durch Schichten aus dasselbem Bindemittel verbindet ist-
und **dass** das genannte Paneel weiterhin aufweist:
(c) Verstärkungmittel (7), die mehrere Verstärkungselementen (7) aufweisen, zum Verstärken des Paneels, wobei die genannten Verstärkungmittel in der inneren Schicht (4) angeordnet sind und die ersten (2,3) und zweiten (5,6) äusseren Schichten verbindenwobei die Verstärkungselementen (7) aus Isolierstoff aus Mineralfasern (7) mit grösserer Dichte bestehen, die eingetaucht und angereichert mit einem Bindemittel sind,
(d) eine zusätzliche Schicht (1) von Glastuch mit kleiner Dichte als die Dichte der Glastuchschichten (2, 3- 5,6), wobei die genannte zusätzliche Schicht an der äusseren Fläche des Paneels angeordnet ist, so dass die genannte zusätzliche Schicht (1) sichtbar während Installation des Paneels an der Unterkunftsbereichen des Schiffes ist, wobei die genannte zusätzliche Schicht (1) mit der ersten äusseren Schicht (2, 3) durch das Bindemittel verbindet ist.

2. Das Paneel gemäss Anspruch 1, wobei das Bindemittel aus 33.33% Magnesia mit einer Reinheit von 91-95%, 24.24% Magnesiumchlorid mit einer Reinheit von 47%, 2.02% Natriumsilikat, und 40.40% Wasser besteht.

3. Das Paneel gemäss Anspruch 1, wobei die Glastuchschichten (2, 3·5,6) miteinander and mit der inneren Schicht (4) durch mehrere Bindemittelschichten verbindet sind, und wobei die genannte zusätzliche Schicht (1) mit einer Fläche versehen ist, die für Färbung geeignet ist oder mit einem feuerbeständigen Dekorationüberzug bedeckt ist, der sichtbar während Installation des Paneels an der Unterkunftsbereichen des Schiffes ist.

4. Das Paneel gemäss Anspruch 1, wobei die genannten Verstärkungsmittel (7) Verstärkungsstreifen sind, die parallel zur der langen Dimension des Paneels und vertikal zur seiner Flache sind, wobei die genannten Mittel mit dem Isolierstoff der inneren Schicht (4) und mit den äusseren Schichten (2, 3·5, 6) des Paneels durch mehrere Bindemittelschichten verbindet sind.

5. Das Paneel gemäss Anspruch 1, wobei die genannten Verstärkungmittel (7) jeden anderen zweckmässigen Verstärkungsstoff aufweisen.

6. Das Paneel gemäss Anspruch 1, weiterhin aufweisend Verbindungmittel zum Verbinden der Paneels zueinander, zum Boden, zu kantigen Elementen, oder zu allgemeinen Paneelstützen für Installation des Paneels an einem Schiff.

7. Das Paneel gemäss Anspruch 1, wobei das genannte Paneel eine Dicke von 25 mm hat.

8. Das Paneel gemass Anspruch 1, wobei das Paneel ein Doppeltdickepaneel mit einer Dicke von 50 mm ist, wobei das Doppeltdickepaneel eine dicken inneren Schicht von Isolierstoff hat.

9. Feuerbeständige Tür aus Paneele gemäss einer der vorhergehenden Asprüchen, aufweisend:
(a) eine ersten äussere starren Schicht (2, 3) und eine zweiten äusseren starren Schicht (5, 6), wobei die ersten und zweiten äusseren starren Schichten (2, 3, 5, 6) an entgegengesetzten Seiten der Tür angeordnet sind, und eine inneren starren Schicht, wobei jede der genannten ersten (2, 3), zweiten (5, 6) und inneren Schichten Glastuchschichten aufweisen, die durch ein Bindemittel verbindet sind
(b) erste und zweite inneren Isolierschichten (4), die Mineralfasern aufweisen, wobei die ersten und zweiten Isolierschichten (4) mit den genannten starren Schichten (2, 3, 5, 6) durch das Bindemittel verbindet sind, wobei die erste innere Isolierschicht (4) zwischen der ersten äusseren starren Schicht (2, 3) und der inneren starren Schicht angeordnet ist, und die zweite innere Isolierchicht (4) zwischen der zweiten äusseren starren Schicht (5, 6) und der inneren starren Schicht angeordnet ist und
(c) mehrere Verstärkungselementen (7), die in die ersten und zweiten inneren Schichten (7) eingebracht sind und die starren Schichten verbinden, wobei die genannten Verstärkungselementen (7) ein Isolierstoff aus Mineralfasern mit grosser Dichte aufweisen, die eingetaucht und angereichert mit einem verstärkenden Bindemittel sind.
wobei das genannte Bindemittel Magnesia, Magnesiumchlorid, Natriumsilikat und Wasser aufweist and kein Magnesiumsulphat enthält.

10. Verfahren zur Herstellung des Paneels gemäss Anspruch 1, wobei das Verfahren ein Kaschierungschritt unter Verwendung einem Kaltverdichtungsprozess aufweist, **dadurch gekennzeichnet dass**
die genannte erste Schicht (2, 3) eine äusserste Glastuchschicht (1) mit kleiner Dichte als die Dichte der anderer äusserer Glasschichten aufweist
und dass das genannte Bindemittel Magnesia, Magnesiumchlorid, Natriumsilikat und Wasser aufweist and kein Magnesiumsulphat enthält.

11. Verfahren zur Herstellung von vorgefertigten oder halbvorgefertigten Schiffunterkunftskabinen, aufweisend:
(a) Erhalten von mehreren Paneelen, aufweisend das Paneel gemäss Anspruch 1. und
(b) Zusammensetzung der Paneele zur Kabine.

12. Verfahren zur Herstellung von vorgefertigten hygienischen Einheiten für Schiffen, aufweisend
(a) Erhalten von mehreren Paneelen, aufweisend das Paneel gemäss Anspruch 1 und
(b) Zusammensetzung der Paneele zur hygienischen Einheit.

13. Verfahren zur Herstellung von feuerbeständigen Klass B-15 Verbindungen zum Verbinden von Vakuumtoilettensystemen, aufweisend:
(a) Erhalten von mehreren Paneelen, aufweisend das Paneel gemäss Anspruch 1. und
(b) Zusammensetzung der Paneele zur Verbindung.

14. Verfahren zur Herstellung von Zimmerdeckeausparungen in einem Schiff, aufweisend:
(a) Erhalten von mehreren Paneelen, aufweisend das Paneel gemäss Anspruch 1. und
(b) Zusammensetzung der Paneele zu Zimmerdeckeausparungen.

## Revendications

1. Panneau résistant aux flammes et isolant du son pour espaces d'hébergement de navire, ledit panneau comprenant:
(a) une première couche extérieure (2, 3) et une deuxième couche extérieure (5, 6), lesdites première (2, 3) et deuxième (5, 6) couches extérieures étant disposées sur les faces opposées du panneau,
(b) une couche intérieure (4) de matériau isolant comprenant des fibres minérales,
**caractérisée en ce que**
chacune desdites couches extérieures (2, 3; 5, 6) consiste en deux couches de tissu en fibres de verre qui sont attachées au moyen d'un matériel liant, ledit matériel liant comprenant de la magnésie, du chlorure de magnésium, du silicate de sodium et de l'eau et étant exempt de sulfate de magnésium;
**en ce que** ladite couche intérieure (4) est attachée à ladite couche extérieure (2, 3; 5, 6) par des couches du même matériel liant;
et **en ce que** ledit panneau comprend en plus:
(c) des moyens de renforcement (7), comprenant une multitude d'éléments de renforcement (7), pour renforcer le panneau, lesdits moyens de renforcement étant disposés dans la couche intérieure (4) et reliant la première (2, 3) à la deuxième (5, 6) couche extérieure; les éléments de renforcement (7) consistant en un matériel d' isolation en fibres minérales de densité supérieure (7), immergées dans et enrichies avec un matériel liant; et
(d) une couche supplémentaire (1) en tissu de fibres de verre de densité inférieure à la densité des couches de tissu de fibres de verre (2, 3; 5, 6), laquelle couche supplémentaire étant disposée sur une surface extérieure du panneau de sorte que cette couche supplémentaire (1) reste visible après l'installation du panneau dans un espace d'hébergement de navire, ladite couche supplémentaire (1) étant liée à la première couche extérieure (2, 3) au moyen du matériel liant

2. Panneau selon la revendication 1, où le matériel liant consiste en 33,33% de magnésie de 91-95% de pureté, 24,24% de chlorure de magnésium de 47% de pureté, 2,02% de silicate de sodium et 40,40% d'eau,

3. Panneau selon la revendication 1, où les couches de tissu de fibres de verre (2, 3; 5, 6) sont liées entre elles et avec la couche intérieure (4) au moyen de couches multiples de matériel liant et où ladite couche supplémentaire (1) est munie d'une surface propre à être peinte ou elle est couverte avec un revêtement décoratif résistant aux flammes qui reste visible dans les espaces d'hébergement du navire après l'installation du panneau.

4. Panneau selon la revendication 1, où lesdits moyens de renforcement (7) sont des bandes de renforcement appliquées parallèlement à la grande dimension du panneau et perpendiculairement à sa surface, lesdits moyens étant liés avec le matériel isolant de la couche intérieure (4) et avec les couches extérieures (2, 3; 5, 6) du panneau par des couches multiples de matériel liant.

5. Panneau selon la revendication 1, où lesdits moyens de renforcement (7) comprennent tout autre matériel de renforcement approprié.

6. Panneau selon la revendication 1, comprenant en plus des moyens de raccordement pour lier les panneaux entre eux, à un plancher, à des éléments d'angle ou à des supports de panneau quelconques pour l'installation du panneau sur le navire.

7. Panneau selon la revendication 1, où ledit panneau a une épaisseur de 25 mm.

8. Panneau selon la revendication 1, le panneau étant un panneau double épaisseur ayant une épaisseur de 50 mm, où le panneau d'épaisseur double contient une couche intérieure épaisse de matériel isolant.

9. Porte résistant aux flammes construite en panneaux selon l'une quelconque des revendications précédentes, comprenant
(a) une première couche extérieure inflexible (2, 3) et une deuxième couche extérieure inflexible (5, 6), lesdites première et deuxième couches extérieures inflexibles (2, 3; 5, 6) étant disposées sur les faces opposées de la porte, et une couche intérieure inflexible, chacune de ces première, deuxième couches et couche intérieure comprenant des couches de tissu des fibres minérales liées avec un matériel liant;
(b) une première et une deuxième couches isolantes intérieures (4) comprenant des fibres de verre, lesdites première et deuxième couches isolantes (4) étant liées auxdites couches inflexibles (2, 3, 5, 6) avec du matériel liant, où la première couche intérieure isolante (4) est disposée entre la première couche extérieure inflexible (2, 3) et la couche intérieure inflexible et la deuxième couche intérieure isolante (4) est disposée entre la deuxième couche extérieure inflexible (5, 6) et la couche intérieure inflexible; et
(c) une multitude d'éléments de renforcement (7), introduits dans la première et la deuxième couche intérieure (4) et reliant les couches inflexibles, lesdits éléments de renforcement (7) comprenant un matériel d' isolation en fibres minérales de grande densité immergé dans et enrichi avec un matériel liant de renforcement,
où ledit matériel liant comprend de la magnésie, du chlorure de magnésium, du silicate de sodium et de l'eau et est exempt de sulfate de magnésium.

10. Méthode de fabrication du panneau de la revendication 1, laquelle méthode comprend une étape de laminage utilisant un processus de compression à froid,
**caractérisée en ce que**
ladite première couche extérieure (2, 3) comprend une couche de tissu de fibres de verre tout à fait extérieure (1) de densité inférieure à la densité des autres couche extérieures en fibre de verre;
et **en ce que**
ledit matériel liant comprend de la magnésie, du chlorure de magnésium, du silicate de sodium et de l'eau et est exempt de sulfate de magnésium.

11. Méthode de fabrication d' une cabine d'hébergement de navire préfabriquée ou semi-préfabriquée, comprenant
(a) la provision d' une multitude de panneaux, y compris le panneau de la revendication 1; et
(b) l'assemblage de la cabine à partir des panneaux.

12. Méthode de fabrication d' une unité sanitaire préfabriquée pour navire, comprenant
(a) la provision d' une multitude de panneaux, y compris le panneau de la revendication 1; et
(b) l'assemblage de l'unité sanitaire à partir des panneaux.

13. Méthode de fabrication d'un raccordement anti-incendie de classe B-15 pour le raccordement de systèmes de toilette à vide, comprenant
(a) la provision d' une multitude de panneaux, y compris le panneau de la revendication 1; et
(b) l'assemblage du raccordement à partir des panneaux.

14. Méthode de fabrication d'un faux plafond dans un navire, comprenant
(a) la provision d' une multitude de panneaux, y compris le panneau de la revendication 1; et
(b) l'assemblage du faux plafond à partir des panneaux.
